

# United States Patent

Sonoda et al.

[15] 3,650,759

[45] Mar. 21, 1972

[54] **SILVER HALIDE EMULSION  
CONTAINING 1,2-GLYCOL AS  
SENSITIZER AND ANTIFOGGANT**

[72] Inventors: Minoru Sonoda; Nobuo Yamamoto; Akikazu Mikawa, all of Kanagawa, Japan

[73] Assignee: Fuji Photo Film Co., Ltd., Ashigara-Kamigun, Kanagawa, Japan

[22] Filed: July 9, 1969

[21] Appl. No.: 840,477

[30] **Foreign Application Priority Data**

July 9, 1968 Japan.....43/48021

[52] U.S. Cl.....96/107, 96/109

[51] Int. Cl.....G03c 1/28, G03c 1/34

[58] **Field of Search**.....96/107, 109

[56] **References Cited**

UNITED STATES PATENTS

3,068,102 12/1962 Chiesa et al. ....96/107

3,294,540 12/1966 Goffe.....96/107

*Primary Examiner*—Norman G. Torchin

*Assistant Examiner*—Won H. Louie, Jr.

*Attorney*—Sughrue, Rothwell, Mion, Zinn & Macpeak

[57] **ABSTRACT**

A photographic silver halide light-sensitive emulsion is enhanced in sensitivity without an attendant increase in fog by addition to the silver halide emulsion of a 1,2-glycol of the general formula



wherein R<sub>1</sub>, R<sub>2</sub> and R<sub>3</sub> represent a hydrogen atom or an alkyl group, and R<sub>4</sub> represents a hydrogen atom, an alkyl group, an aryl group, an alkoxyalkyl group, an aryloxyalkyl group, or an allyloxyalkyl group.

**11 Claims, No Drawings**



mide) was added 2,3-butanediol (Compound (b)). A second and a third emulsion were likewise prepared incorporating 1,2-butanediol (Compound (c)), and pinacol (Compound (f)) respectively. The resulting silver halide emulsions were subjected to a second ripening by sulfur and gold sensitizations at 52°C. Then, after adding a suitable amount of chromium alum and saponin, the coating compositions thus prepared were applied to cellulose acetate films so that the amount of silver coated became 45 mg./100 sq. cm. and dried. For comparison, a control sample was prepared by the aforesaid procedure but without adding the compound of this invention.

The photographic light-sensitive films thus prepared were exposed by using a NSG-II sensitometer and developed for 7 minutes at 20°C. in a developer having the following composition:

|                            |         |
|----------------------------|---------|
| p-Aminophenol              | 2.0 g.  |
| Sodium sulfite (anhydrous) | 100 g.  |
| Hydroquinone               | 5 g.    |
| Borax                      | 2.0 g.  |
| Water to make              | 1 liter |

The results are shown in the following table, in which the sensitivity shown is a relative value calculated from the exposure amount giving a density of fog + 0.3 assuming the sensitivity of the control sample ripened for 50 minutes being 100.

| Compound  | Amount* | Ripening Period |         |         |      |     |      |
|-----------|---------|-----------------|---------|---------|------|-----|------|
|           |         | 50 min.         | 65 min. | 80 min. | A    | B   | A    |
| None      |         |                 |         |         |      |     |      |
| (Control) | —       | 100             | 0.08    | 131     | 0.16 | 136 | 0.33 |
| (b)       | 15.3    | 110             | 0.05    | 144     | 0.07 | 151 | 0.11 |
| (c)       | 15.3    | 113             | 0.06    | 143     | 0.07 | 158 | 0.10 |
| (f)       | 20.0    | 113             | 0.06    | 144     | 0.07 | 150 | 0.10 |

\*Concentration by g./mole of silver iodobromide; A: sensitivity; B: fog.

From the above results, it is seen that the photographic silver halide emulsion containing the additive of this invention had a high sensitivity and gave less formation of fog.

### EXAMPLE 2

Two separate silver iodobromide emulsions were prepared (1.5 mole percent AgI and 150 g. of gelatin per one mole of silver iodobromide) for high-speed X-ray photographic film, and 1,2-hexanediol (Compound (g)), and 1-phenyl-1,2-ethanediol (Compound (h)) were added to the respective emulsions. These emulsions were then subjected to second ripening by sulfur-gold sensitization at 53°C. after adding a suitable amount of chromium alum and saponin, the silver halide emulsions thus prepared were applied to a cellulose acetate film so that the amount of silver applied became 55 mg./100 sq. cm. and dried. For comparison, a control sample was prepared by the same procedure as above without employing the compound of this invention. The photographic films thus obtained were exposed by using a NSG-II sensitometer and developed for 4 minutes at 20°C. in a developer having the composition as follows:

|                              |         |
|------------------------------|---------|
| p-Aminophenol                | 4.0 g.  |
| Sodium sulfite (anhydrous)   | 60.0 g. |
| Hydroquinone                 | 10.0 g. |
| Sodium Carbonate (anhydrous) | 53.0 g. |
| Potassium Bromide            | 2.5 g.  |
| Water to make                | 1 liter |

The results are shown in the following table, in which the sensitivity shown is a relative value calculated from the exposure amount giving the density of fog + 0.3 assuming the sensitivity of the control sample ripened for 125 minutes being 100.

| Compound  | Amount* | Ripening Period |      |          |      |     |      |
|-----------|---------|-----------------|------|----------|------|-----|------|
|           |         | 125 min.        | min. | 155 min. | A    | B   | A    |
| None      |         |                 |      |          |      |     |      |
| (Control) | —       | 100             | 0.11 | 126      | 0.13 | 140 | 0.17 |
| (g)       | 18.3    | 129             | 0.06 | 148      | 0.08 | 160 | 0.12 |
| (h)       | 11.7    | 111             | 0.09 | 133      | 0.10 | 155 | 0.13 |

\*Concentration by g./mole of silver iodobromide; A: sensitivity; B: fog.

From the above results it is seen that the photographic silver halide emulsion containing the additive of this invention has a higher sensitivity and less fog than the control sample.

### EXAMPLE 3

To separate gelatino silver iodobromide emulsions (7 mole percent AgI and 200 g. of gelatin per one mole of silver iodobromide) for high speed negative photographic film subjected to sulfur sensitization and gold sensitization, were added 3-m-octyloxy-1,2-propanediol (Compound (k)), 3-aryloxy-1,2-propanediol (Compound (l)), 3-phenoxy-1,2-propanediol (Compound (m)), and 3-(2-methoxy)phenoxy-1,2-propanediol (Compound (o)) directly before coating, respectively. After further adding a suitable amount of chromium alum and saponin, the resulting silver halide emulsion was applied to a cellulose acetate film and dried. For comparison, a control sample was prepared by the same procedures as above without employing the additive of this invention.

These photographic films were exposed and developed as in Example 1, the results of which are shown in the following table in which the sensitivity was shown assuming the relative sensitivity of giving the density of fog + 0.3 being 100.

| Compound  | Amount* | Sensitivity                |             |       | Gamma | Fog |
|-----------|---------|----------------------------|-------------|-------|-------|-----|
|           |         | g./mole silver iodobromide | Sensitivity | Gamma |       |     |
| None      |         |                            |             |       |       |     |
| (Control) | —       | 100                        | 0.70        | 0.70  | 0.20  |     |
| (k)       | 9.4     | 113                        | 0.83        | 0.83  | 0.09  |     |
| (l)       | 6.6     | 112                        | 0.80        | 0.80  | 0.10  |     |
| (m)       | 8.4     | 113                        | 0.83        | 0.83  | 0.09  |     |
| (o)       | 9.9     | 113                        | 0.81        | 0.81  | 0.09  |     |

\*Concentration

From the above results, it will be understood that the photographic silver halide emulsion of this invention prepared above had a high sensitivity and gave less fog.

What is claimed is:

1. A silver halide photographic emulsion containing a compound represented by the general formula



wherein R<sub>1</sub>, R<sub>2</sub> and R<sub>3</sub> each represents one member selected from the group consisting of a hydrogen atom and an alkyl group, and R<sub>4</sub> represents one member selected from the group consisting of a hydrogen atom, an alkyl group, an aryl group, an alkoxyalkyl group, an aryloxyalkyl group and an allyloxyalkyl group.

2. The silver halide photographic emulsion as claimed in claim 1 wherein said compound is selected from the group consisting of 2,3-butanediol, 1,2-butanediol, pinacol, 1,2-hexanediol, 1-phenyl-1,2-ethanediol, 3-m-octyloxy-1,2-propanediol, 3-aryloxy-1,2-propanediol, 3-phenoxy-1,2-propanediol and 3-(2-methoxy)phenoxy-1,2-propanediol.

3. The silver halide photographic emulsion as claimed in claim 1 wherein the amount of said compound is in the range

of from 2 to 100 g. per mol of silver halide.

4. A process for preparing silver halide photographic emulsion which comprises adding a compound represented by the general formula



wherein  $R_1$ ,  $R_2$  and  $R_3$  each represents one member selected from the group consisting of a hydrogen atom and an alkyl group, and  $R_4$  represents one member selected from the group consisting of a hydrogen atom, an alkyl group, an aryl group, an alkoxyalkyl group, an aryloxyalkyl group and an allyloxyalkyl group, to a physically ripened silver halide emulsion added at the beginning of chemical ripening.

5. A photographic silver halide light-sensitive element comprising a support having coated thereon at least one silver halide emulsion layer containing a compound represented by the general formula



wherein  $R_1$ ,  $R_2$  and  $R_3$  each represents one member selected from the group consisting of a hydrogen atom and an alkyl group, and  $R_4$  represents one member selected from the group consisting of a hydrogen atom, an alkyl group, an aryl group, an alkoxyalkyl group, an aryloxyalkyl group and an allyloxyalkyl group.

6. The photographic silver halide light-sensitive element as claimed in claim 5 wherein said compound is selected from the group consisting of 2,3 butanediol, pinacol, 1,2-hexanediol, 1-phenyl-1,2-ethanediol, 3-m-octyloxy-1,2-propanediol and 3-phenoxy-1,2-propanediol.

7. The silver halide photographic emulsion as claimed in claim 1, wherein the amount of said compound is in the range of from 5 to 50 g. per mol of silver halide.

8. The photographic silver halide light-sensitive element as

claimed in claim 5, wherein said compound is present in an amount of from 2 to 100 g. per mol of silver halide.

9. The photographic silver halide light-sensitive element as claimed in claim 8, wherein said compound is present in an amount of from 5 to 50 g. per mol of silver halide.

10. The silver halide photographic emulsion as claimed in claim 1, wherein said compound is selected from the group consisting of



25 11. The photographic silver halide light-sensitive element as claimed in claim 5, wherein said compound is a member selected from the group consisting of



\* \* \* \* \*

45

50

55

60

65

70

75